

# UNITED STATES PATENT OFFICE.

JEGOR ISRAEL BRONN, OF ROMBACH, GERMANY, ASSIGNOR OF ONE-HALF TO THE FIRM  
OF ROMBACHER HÜTTENWERKE, OF ROMBACH, GERMANY.

## MANUFACTURE OF STEEL.

1,156,051.

Specification of Letters Patent. Patented Oct. 12, 1915.

No Drawing.

Application filed December 2, 1912. Serial No. 734,614.

*To all whom it may concern:*

Be it known that I, JEGOR ISRAEL BRONN, a citizen of the German Empire, and resident of Rombach, Lorraine, Germany, have 5 invented new and useful Improvements in the Manufacture of Steel, of which the following is a specification.

The invention relates to a novel process of making steel, and comprises, first, forming a purified and decarburized molten main charge of iron, second, forming a subsidiary charge, preferably of purified molten iron, third, dissolving in said secondary molten charge the necessary additional elements in 15 proper proportion for the steel to be made from the main charge, and finally mixing the main and subsidiary charges while in molten condition. Otherwise stated the additions which it is desired to make to the 20 bath of a refined iron for the purpose of deoxidation, desulfurization, carburation, elimination of gas or alloying with other metals, are first dissolved in liquid iron contained in a separate furnace, and then the 25 resulting dilute molten solution of the said additions in the molten iron is poured together with the bath of refined iron into the casting ladle wherein they become mixed together. When the refining furnace is so 30 constructed that the slag covering can be removed from the main iron bath (for instance in tilting furnaces), the molten solution of iron may also be added to the main bath contained in the refining furnace after 35 having previously removed the slag covering from the latter. It is advisable to use refined (soft) iron of the greatest possible purity as the solvent in order that no undesirable constituents shall be added to the 40 main iron bath through the medium of the solvent. Now since such refined iron is always available in the molten state in steel-works, it is advisable, for the sake of saving the cost of remelting, to charge the dissolving furnace (which can be heated by gas, 45 oil, or electricity) with such liquid iron, and to dissolve therein the desired additions (for instance carbon in the form of powdered coke, coke briquets, or carburite, or metals such as manganese, silicon, titanium, vanadium, tungsten, chromium) either in the 50 pure state or in the form of ferro-alloys mixed in the desired proportions. By this means a solution is produced containing one

or more of these constituents in exactly determined quantities and groupings, and this solution is mixed with the main bath of refined iron. This improved method will now be described more fully with reference to examples and will be compared with existing methods. For instance, for the purpose of effecting carburation according to the new process, liquid iron is saturated with carbon at the highest possible temperature in a dissolving furnace by the addition of 55 coke, carbon briquets, or other carbonaceous mixtures, thus producing a molten solution of iron containing exactly determinable quantities of carbon.

To prepare a charge of steel having a certain percentage of carbon, the corresponding quantity of iron-carbon is taken from the dissolving furnace and is introduced while still liquid into the steel forming charge that is to be prepared, care being 70 taken to remove the slag covering therefrom. For instance, if it is desired to make a 10 ton charge of Thomas, Bessemer, or Martin steel containing 0.6% of carbon, that is, a 75 total content of

$$10 \times 6 = 60 \text{ kgs.}$$

of carbon, it will be necessary to take

$$\frac{60}{54} = 1.11 \text{ tons}$$

80

of molten metal from the dissolving furnace because each ton of 0.6% carbon steel contains

$$60 - 6 = 54 \text{ kgs.}$$

90

of carbon. Thus the improved process admits of production with certainty, from ordinary Bessemer, Thomas, or Martin ingot iron, at a very low cost, pure carbon steel of extraordinarily uniform quality 95 even when dealing with very large charges.

Heretofore when it has been desired to produce carbon steel it has been usual to add the carbonaceous substances (coke, coke briquets and the like) to the ingot iron in the Martin furnace or electric furnace, with the resultant disadvantage that the carbon is taken up only in part by the iron bath, another part of the carbon being taken up by the slag covering, while a further part 100 is lost by direct combustion. The absorption of the carbon by the slag is usually accomplished by several reactions as a result

of which the constituents of the slag, more especially phosphorus, are reduced and incorporated again in the iron bath. That method occasions great loss of time because the operator must wait until the carbon has become dissolved and it is impossible to know beforehand exactly how much carbon is taken up by the iron, and further there is the risk that the noxious constituents of the slag may be taken up again by the iron. Now in order to avoid these subsidiary reactions it has also been proposed to introduce the carbon subsequently with the ingot iron into the casting ladle. It is however obvious that that method cannot yield a homogeneous product of uniform quality and composition.

Another example:—For the purpose of making manganese steel according to the improved process, manganese or ferromanganese is dissolved in the liquid iron contained in a dissolving furnace, and the solution is mixed with the main charge of the steel to be made. In order to make a manganese-carbon steel containing a given percentage of carbon and manganese, the corresponding quantity of carbon is dissolved in the dissolving furnace at the same time as the ferro-manganese. It has heretofore been usual to make such steels by means of spiegeleisen. In such a case a charge of about 25 tons of medium hard steel will require about 2000 kgs. of spiegeleisen containing 10% of manganese and about 4.5% of carbon. In order to obtain the requisite 200 kgs. of manganese and 90 kgs. of carbon the steel maker will have to buy 1700 kgs. of outside iron which will naturally cost him much more than the iron he makes himself, and he will have in addition to pay ten times the cost of carriage. To obtain the iron in the molten state it will also be necessary to melt down the whole 2000 kgs. which will entail a great consumption of fuel, or, in the case of an electric furnace, a great consumption of electrical energy. Now with the improved process the state of affairs is quite different:—Here, since, as already stated, every steel maker always has liquid ingot iron available in large quantities, about 1750 kgs. of this ingot iron are charged while liquid into the dissolving furnace 250 kgs. of ferro-manganese with 80% of manganese and also if required the desired quantities of carbon, ferro-silicon and the like are dissolved with application of heat and the solution is now ready for use. The necessary consumption of heat or energy is thus reduced to about  $\frac{1}{8}$  of the formerly required amount. There is also the further advantage that the solutions can be of any desired concentration without being tied to the use of the stock brands of spiegeleisen, and that iron solutions which are to con-

tain no constituent other than manganese for instance, or which are to contain a number of reagents together (for instance carbon, silicon, etc.) can be produced with any desired groupings or proportions of such constituents. If as was often the case heretofore spiegeleisen was added to the previously refined steel charge the same disadvantages were experienced as in the process of carburation in the furnace but in a very much greater degree, namely delay in the finishing of the charge, subsidiary reaction with the slag covering so that a part of the valuable manganese was lost in the slag, and moreover the constituents reduced from the slag entered as impurities in the steel bath. The improved process is carried out in an analogous manner when instead of or in addition to carbon and manganese it is desired to add other metals to the steel charge either for the purpose of refining it or producing alloys. For instance if it is desired to make a steel containing chromium, nickel, manganese and carbon, the liquid iron present in the dissolving furnace is mixed with these ingredients in the desired proportions, and when the whole mass has become molten the solution is mixed with the steel charge to be made. The iron contained in the dissolving furnace serves as above stated, as a solvent vehicle for the reagents that are to be added. The purer this solvent the greater the freedom of the operator in grouping the subsidiary constituents. In some cases however a perfect purity is of less importance as regards the solvent iron. If it is desired for instance to make the carbon steels hereinbefore described, foundry cast iron of the greatest possible purity containing already about 2.5% of carbon may be employed instead of the soft ingot iron above referred to.

The advantages of the improved process are due to the simultaneous coöperation of several factors the chief of which are the following:—

(a) The different additions are added to the steel bath in a manner which precludes the loss of the active constituents, for instance by volatilization, formation of slag and oxidation such as often occurs with existing methods.

(b) The ease with which steels of any desired composition and grouping of the constituents may be produced, for instance, carbon steels which are almost free from manganese or steels poor in carbon but rich in manganese. Heretofore this has been very much more difficult because for instance in spiegeleisen as also in ferro-manganese the proportion between the contained percentage of manganese and the contained percentage of carbon is almost fixed and this mutual dependence of the two elements affects also the finished products.

- (c) By this means it is possible to manufacture steels of complex composition with heretofore unattainable exactness and precision.
- 5 (d) The molten state of the subsidiary charge guarantees the uniform action and distribution of the several constituents in the main charge.
- (e) By the use of a quantity of highly heated metal, many times greater than the quantity of the constituent to be added, the risk of congealing during the various manipulations is avoided. Thus, for instance, heretofore in making vanadium steel and 15 titanium steel usually only a very small percentage of these metals or their alloys was added in solid form to the steel charge, it being assumed that the said percentage will be dissolved and become uniformly distributed throughout the charge without residue. Such is however not the case and this is no 20 doubt the cause of many failures that have been experienced with these steels. Even if it were attempted to melt these constituents beforehand as is often done now in the case of ferro-manganese, success is not certain, because since only small quantities of say 20-30 kgs. are dealt with in this case such small quantities of molten metal would 25 congeal on the way from the melting furnace to the place of use, while the melting of such valuable metals is attended by heavy loss in consequence of their great tendency to oxidation, (formation of slag).
- (f) The addition of a relatively large quantity of highly heated molten iron with the constituents dissolved therein not only does not withdraw any heat from the steel charge, as is the case when the additions are 30 thrown in solid but even adds an increment 40 of heat to the steel charge.

What I claim is—

1. The process of manufacturing steel which consists in introducing the required additions in solid form into a quantity of 45 liquid iron, and mixing the solution so obtained with the refined molten iron constituting the main steel making charge.
2. The process of manufacturing steel which consists in melting a quantity of iron, 50 adding to it manganese or a manganese alloy and carbon in desired proportions, in solid form and mixing the solution so obtained with the main charge of molten refined iron.
3. The process of manufacturing steel which consists in melting a quantity of refined iron, adding to it carbon in desired proportions and mixing the solution so obtained with the main charge of molten refined iron.
4. The process of making steel, which consists in refining and decarburizing a main charge of iron in a suitable furnace, 55 forming a subsidiary charge by introducing in solid form and dissolving the additional constituents of the ultimate steel in proper proportions in a bath of molten refined iron, and mixing the main and subsidiary charges while in a molten state.

In testimony, that I claim the foregoing as my invention, I have signed my name in presence of two witnesses, this 20 day of November, 1912.

JEGOR ISRAEL BRONN.

Witnesses:

IDA ALLMANN-BRONN,  
JACOB SCHMIDT.